

## UNITED STATES PATENT OFFICE.

CHARLES B. BELKNAP, OF HIGHLAND PARK, MICHIGAN.

## HYDROCARBON FUEL AND METHOD OF MAKING THE SAME.

No Drawing.

Application filed August 29, 1918. Serial No. 251,899.

*To all whom it may concern:*

Be it known that I, CHARLES B. BELKNAP, a citizen of the United States of America, residing at Highland Park, in the county of Wayne and State of Michigan, have invented certain new and useful Improvements in Hydrocarbon Fuel and Methods of Making the Same, of which the following is a specification.

10 This invention relates to hydrocarbon fuel and refers more particularly to hydrocarbon fuel such as is used in automobiles or other internal combustion engines.

15 Among the objects of the invention is to produce a homogenized mixture of hydrocarbon fuel, such as kerosene or gasoline, with water and either with or without a third substance. The invention also resides in the process of producing the fuel and 20 the fuel itself and in the process of operating an internal combustion engine, whereby there is used as a liquid fuel a homogenized mixture of gasoline, kerosene or other hydrocarbon oils or other liquid 25 fuel with water or other substance.

It has heretofore been proposed to increase the efficiency of internal combustion engines by injecting into the manifold or other part of the engine a steam vapor which 30 will not only prevent carbon in the engine, but will give a smoother running and also increase the efficiency of the engine. Such arrangement, however, is commercially objectionable, owing to the necessity of maintaining a separate liquid supply for the water as well as for the fuel, and the present invention particularly contemplates the producing of a fuel in which the gasoline, kerosene or the like is permanently mixed 35 with the water.

In order to produce this fuel I preferably employ a mixture of kerosene, gasoline and water which, after being mixed by agitation to produce either an emulsified or other 40 state, is run through a homogenizing valve at an extremely high pressure, as for instance 4000 pounds to the square inch. One formula I have found to be satisfactory is to employ 9% water, 40% kerosene, 50% 45 gasoline and 1% emulsifying agent. It is understood that I do not limit myself to

these proportions as I may vary them within wide ranges to produce the desired product. The pressure given, however, is merely illustrative and may be raised or lowered 55 depending upon the qualities of the material being treated and the product desired. Also in some cases it may be necessary to mix with the oil and water an emulsifying substance and the mixture is preferably run 60 through the valve while in a heated state say, at a temperature between 100 and 200° F. so as to produce a larger percentage of permanent mixture.

One type of apparatus which may be employed for producing this fuel is shown in the patent to Gaulin No. 756,953, although the invention in its broader aspects is not limited to the use with any particular homogenizing machine. The resultant product 70 is then vaporized and mixed with air in a manner similar to that used with ordinary gasoline or kerosene fuels.

By the phrase "homogenized mixture" as employed in the claims is meant a mixture 75 having a high resistance to separation and like general characteristics similar to that of a mixture produced by the use of the homogenizing valve above mentioned.

What I claim as my invention is:— 80

1. A fuel, comprising a homogenized emulsion of hydrocarbon liquid and water, the water content of which is dispersed throughout the emulsion in excess of the normal mixing capacity of the emulsion. 85

2. The method of producing fuel which comprises emulsifying hydrocarbon liquid and water, and increasing the dispersion of the water throughout the emulsion above the normal mixing capacity of the emulsion 90 by passing the emulsion under relatively high pressure through a homogenizing process.

3. An emulsion fuel capable of explosion in an internal combustion engine, comprising a hydrocarbon oil and water, said mixture having been stabilized by homogenizing action. 95

In testimony whereof I affix my signature.

CHARLES B. BELKNAP.